# EUROPEAN PATENT SPECIFICATION

(11) **EP 1 828 440 B1**
(45) Date of publication and mention of the grant of the patent: **19.09.2012**
(21) Application number: 05819032.3
(22) Date of filing: 14.12.2005
(51) Int. Cl.: C25D 5/18

(54) **PULSE-PLATING METHOD AND APPARATUS**
PULSMETALLABSCHEIDUNGSVERFAHREN UND -VORRICHTUNG
PROCEDE ET APPAREIL D'ELECTRODEPOSITION SOUS IMPULSIONS

(30) Priority: 14.12.2004 SE 0403047
(43) Date of publication of application: 05.09.2007
(73) Proprietor: Polymer Kompositer I Göteborg, 431 53 Mölndal (SE)
(72) Inventor: REMGÅRD, Anders, S-431 49 Mölndal (SE)
(74) Representative: Valea AB
(86) International application number: PCT/SE2005/001928
(87) International publication number: WO 2006/065220

(56) References cited:
- EP-B1- 0 868 545
- WO-A1-99/18266
- WO-A2-02/33150
- GB-A- 1 396 436
- GB-A- 2 214 520
- US-A- 4 436 591
- US-A- 4 608 138
- US-A- 4 666 567
- US-A1- 2001 023 830
- US-A1- 2002 104 755
- US-A1- 2004 011 654

## Description

### Field of the invention

The present invention relates to a method and apparatus for pulse-plating. A novel pulse sequence is also disclosed.

### Background

Galvanic plating of electrically-conducting materials and objects is well-known and has been used for many years to provide conductive or protective layers of metal on an object. In the simplest form of galvanic plating, the object to be plated is connected to an electric circuit such that it acts as an anode, and is immersed in a bath containing a solution of metal ions. A counter electrode is also connected to the circuit and is also immersed in the bath. An electric current is supplied to the circuit, and the object becomes plated with metal.

More recent developments in the field of galvanic plating allow the thickness, conductivity and brightness of the layer to be varied. Multiple layers or layers comprising a mixture of metals may also be introduced. Modern galvanic plating can further introduce visually attractive features to the object.

US patent application US2004/0140219 discloses a system and method for pulse current plating. The current is varied from a first level to a second level to provide for differing rates of deposition of a conductive material on the substrate. A relaxation period is included in the pulse sequence to allow the conductive material to reach equilibrium.

US patent number 6,750,144 discloses a method for electrochemical metallization and planarization of semiconductor substrates. A series of plating steps is used, each one comprising a train of pulses. The method is used for filling recesses of different sizes on semiconductor substrates.

The article "Plating with Pulsed and periodic-Reverse Current" By Tai-Ping Sun, C.C. Wan & Y. M.Shy, in Metal Finishing from May 1979 discusses the effects of current wave forms on film structure, surface morphology and microhardness.

A particular challenge for practitioners of galvanic plating is to obtain a layer of even thickness, especially when the object to be coated has a complicated or delicate structure. Electric field variations across the surface of an object give rise to variations in the thickness of the plating, particularly where sharp angles on the object's surface concentrate the electric field. At these points, the thickness of the plating is also found to increase. With increasing miniaturisation, problems arise as plating extends to areas where it is not desired, often causing short-circuits.

One solution to the problem of uneven plating is to add chemicals known as "levellers" to the bath. These promote even plating, but may be expensive, increase the need for waste stream purification or adversely affect the quality of the plating.

Severe problems arise when the object to be plated contains cavities, particularly deep cavities. It is particularly difficult to provide a layer of even thickness inside such cavities. Galvanic plating using DC tends to deposit a thick layer of metal around the opening of the cavity and little or no plating occurs at the deeper surfaces of the cavity.

### Summary of the invention

The present invention provides a method for pulse-plating which addresses the disadvantages of the prior art. Particularly, it allows even, uniform coatings to be applied, even deep inside cavities in the object.

The invention relates to a method for plating a object with a metal coating, said method comprising the steps of:
a. bringing the object into contact with a solution comprising metal ions;
b. bringing a counter electrode into contact with said solution comprising metal ions;
c. connecting an electrical circuit between the object and the counter electrode;
d. applying a constant DC current I₁ to the electrical circuit for a time period t₁ so as to provide a current density A₁ on the surface of the object so that the object becomes plated with a metal coating;
e. applying a second constant DC current I₂ in the opposite direction as I₁ to the electrical circuit for a time period t₂ so as to provide a current density A₂ on the surface of the object;
f. applying a third constant DC current I₃ in the same direction as I₁ to the electrical circuit for a time period t₃ so as to provide a current density A₃ on the surface of the object; wherein steps e. and f. may take place in either order;
g. repeating steps e. and f., and optionally step d, until the object is plated with the required profile of the metal,
wherein steps e and f take place in immediate succession, such that time periods t₂ and t₃ are sequential.

### Brief description of the Figures

Figure 1 is a graphical illustration of the variation of current according to the present invention.
Figure 2 is a graphical Illustration of the variation of current according to the present invention when steps d, e and f are repeated sequentially.
Figure 3 is a plan view of a base station filter.

### Detailed description

The term "cavity" is used in the present context to mean a part of the object in which material been drilled, moulded, gouged or otherwise removed from the object to leave an empty space. It includes those cases in which holes are made completely through an object from one surface to another.

As mentioned above, the invention relates to a method for plating a object with a metal coating, said method comprising the steps of: a) bringing the object into contact with a solution comprising metal ions; b) bringing a counter electrode into contact with said solution comprising metal ions; c) connecting an electrical circuit between the object and the counter electrode; d) applying a constant DC current I₁ to the electrical circuit for a time period t₁ so as to provide a current density A₁ on the surface of the object so that the object becomes plated with a metal coating; e) applying a second constant DC current I₂ in the opposite direction as I₁ to the electrical circuit for a time period t₂ so as to provide a current density A₂ on the surface of the object; f) applying a third constant DC current I₃ in the same direction as I₁ to the electrical circuit for a time period t₃ so as to provide a current density A₃ on the surface of the object; wherein steps e. and f. may take place in either order; g) repeating steps e. and f., and optionally step d, until the object is plated with the required profile of the metal, wherein steps e and f take place in immediate succession, such that time periods t₂ and t₃ are sequential.

Figure 1 illustrates an embodiment of the invention in its most simple form, and shows a graph of how the applied current varies with time. A DC current I₁ is applied for a time t₁ (step d, above), followed by a short reversal of current to I₂ for a time t₂ (step e, above). The current is reversed again to a value I₃ for a time t₃ (step f, above). As can be seen from Fig. 1, currents I₂ and I₃ (steps e and f, above) are repeated until the required profile of the metal is obtained. It is not necessary to begin the pulse-plating sequence with the reverse current (I₂); rather I₃ can be applied first (i.e. steps e. and f. may take place in either order).

Figure 2 shows how the applied current varies with time in an embodiment of the invention in which, after steps e and f have been repeated a number of times, step d is repeated (application of a current I₁).

In the above method, A₁ is between 0.1 and 5.0 amperes/dm², preferably between 0.2 and 2.0 amperes/dm² and more preferably between 0.25 and 0.75 amperes/dm². A₂ is generally greater than A₃. For example, A₂ may be at least 1.5 times greater, at least 1.7 times greater, at least 2 times greater or at least 3 times greater than A₃. A₂ is between 0.5 and 5.0 amperes/dm², preferably between 0.5 and 2.0 amperes/dm² and more preferably between 0.5 and 1.75 amperes/dm². Furthermore, A₃ is between 0.5 and 5.0 amperes/dm², preferably between 0.5 and 2.0 amperes/dm² and more preferably between 0.5 and 1.5 amperes/dm².

The length of the time period t₁ is adjusted so that the initial coating of metal reaches the desired thickness. For example, t₁ may be between 10 minutes and 2 hours, preferably between 20 minutes and 1.5 hours, more preferably around 50 minutes.

It is preferred that t₃ is less than t₂. For example, t₃ may be less than 80% of t₂, preferably less than 70% of t₂, most preferably less than 55% of t₂. The time period t₂ is between 0.2ms and 10ms, preferably between 1 and 5 ms and more preferably between 1.5 and 2.5ms. Time period t₃ is between 0.1 ms and 5 ms, preferably between 0.5ms and 2.5ms and more preferably between 0.75ms and 1.25ms.

If a time delay is introduced between I₂ and I₃, the method will not work. The process is very sensitive to changes in pulse lengths and time durations between pulses. In a particular embodiment, it is important that the time periods t₂ and t₃ are the same length when steps e. and f. are repeated.

The current (I) is applied such that the desired current density (A) on the surface of the object can be obtained. The surface area is always important for platers and if no computer-calculated values exist, one has to calculate the surface manually from the actual geometry of the object. The surface area is defined as the part of the component to be plated. The current density is defined as the total current divided by the total surface area to be plated.

The method functions without the use of chemical additives known as "levellers". The method is best suited in those cases where the object contains one or more cavities. It is particularly effective for those cavities which are deeper than they are wide, i.e. wherein the aspect ratio for the cavity, as defined by the ratio between the diameter (D) and the depth (L) of the largest cylinder which fits in the cavity, is between 0.25 and 3 inclusive, preferably between 0.5 and 2.5 inclusive, more preferably 0.75 and 2 inclusive.

As illustrated in Figure 3, for a cavity with an aspect ratio of 1, application of a 3 micron layer of silver or copper to the bottom of a cavity through conventional DC-plating will result in at least 3-4 times this depth of metal on the top sides of the cavity. This can be avoided with the method of the present invention.

The value for I₁ is selected in order to reach the best possible coverage and metal build up in the bottom of the cavity. A typical value is around 0.5 A/dm². The best coverage is achieved with DC-plating but the best levelling is achieved with pulse plating. The values of I₂ and I₃ are chosen depending on what one would like to achieve. By combining these two features, in subsequent steps, it's possible to have a thicker layer in the bottom then on the edges of the cavity.

The method according to the present invention allows the cavity to be selectively etched a predetermined distance from the plane defining the opening of the cavity, without the use of a mask. Alternatively, appropriate use of the method allows the cavity to be selectively etched a predetermined distance from the deepest point of the cavity, without the use of a mask. Examples of predetermined distances which might be desired are 50 % or 75 % of the depth of the cavity. By changing the current densities and ratios for I₂ and I₃, it is possible to control how deep in the cavity the etching takes place, how fast the etching proceeds and the resulting thickness profile of the etched metal layer. Through choice of the current and time it is possible for a cavity to be plated in e.g. only the lower half, or alternatively only in the upper half. By "etching" is meant the removal of metal which has been plated.

For plating deep cavities, the method involves the consecutive steps of:
1. Plating the cavities until the requested thickness is reached in the bottom of the cavity, with DC current at a low current density. For plating of copper, to obtain a typical base station filter with a minimum thickness of 3 micron in the bottom, this DC-plating will be performed at a current density (A₁) of 0.5 A/dm² under 35 minutes (t₁).
2. Applying PRC, (Pulse Reverse Current), with a direction opposite to that of the initial current, i.e. etching for levelling the metal layer. For a typical filter described above, the method typically involves a forward pulse length (t₃) of 1.0 ms and a current density (A₃) of 1.0 A/dm² and a reverse pulse length (t₂) of 2.0 ms and a current density (A₂) of 1.7 A/dm². For copper plating of a filter as under point 1, this pulse plating (repeating steps e. and f. of the method) will go on for approx. 8-10 min.

Under the inventive current/time profile used for etching, the pulse plating step will only affect the metal layer in the bottom of the cavity very little.

Suitable metals for use In the present method are Ag, Au, Cu, Ni, Cr and Zn. Typically, the metal ion is present in a concentration of between 0.1 g/l and 500 g/l. The metals are present in ionic form, having a one or more counter ions which may be selected from the group comprising sulphate, nitrate, chloride, fluoride, bromide, iodide, phosphate, hydroxide, cyanide and/or pyrophosphate.

In one embodiment, the solution comprising metal ions additionally contains one or more surfactants. Preferably, these are selected from the group consisting of non-ionic surfactants, and are more preferably substituted alkylene oxide compounds. In a most preferred embodiment, the surfactant is nonylphenol ethoxylate. Commonly, the surfactant is present in a concentration of between 0.01 g/l and 10g/l, preferably between 0.1g/l and 1g/l and more preferably between 0.1g/l and 0.3g/l. The use of polyoxyalkylene compounds will keep the brightness dose to what is achieved after DC-plating.

The solution comprising metal ions may additionally contain a polymer. The polymers to be used in the bath are preferably oxyethylene-based (homo, graft and block copolymers), and more preferably polyethyleneglycol with an average molecular weight between 100 and 4000. The polymers are usually present in a concentration ranging from 0.01g/l to 10.0g/l inclusive, preferably from 0.01g/l to 1.0g/l inclusive, more preferably from 0.10g/l to 1.0g/l.

Any object may be plated by the method described herein. Objects which are of particular interest are microwave components and base station filters. The objects which can be plated by the method of the present invention can be made of aluminium, zinc, steel including stainless steel and polymers.

An apparatus for carrying out the method described herein, said apparatus may comprise:
a. a container suitable for containing a solution comprising metal ions,
b. a solution comprising metal ions,
c. a current source comprising means for varying the current I under a time t as set out herein,
d. electrical connections, and
e. a counter electrode.

A pulse sequence for carrying out the above-described method, may comprise
a. applying a constant DC current I₁ to the electrical circuit for a time period t₁ so as to provide a current density A₁ on the surface of the object so that the object becomes plated with a metal coating;
b. applying a second constant DC current I₂ in the opposite direction as I₁ to the electrical circuit for a time period t₂ so as to provide a current density A₂ on the surface of the object;
c. applying a third constant DC current I₃ in the same direction as I₁ to the electrical circuit for a time period t₃ so as to provide a current density A₃ on the surface of the object;
d. repeating steps e. and f., and optionally step d, until the object is plated with the required profile of the metal
wherein A₁, A₂, A₃, t₂ and t₃ are as defined above. Particularly, it is of interest that the time periods t₁, t₂ and t₃ in the above-mentioned pulse sequence are sequential.

The present invention also concerns a list of computer-readable instructions, said instructions when loaded into the memory of a processor connected to a DC power supply cause the processor to vary the current I of the power supply according to the above-mentioned pulse sequence.
A computer-readable instruction for carrying out the pulse-plating sequences of the method may comprise the following directions:
a. applying a constant DC current I₁ to the electrical circuit for a time period t₁ so as to provide a current density A₁ on the surface of the object so that the object becomes plated with a metal coating;
b. applying a second constant DC current I₂ in the opposite direction as I₁ to the electrical circuit for a time period t₂ so as to provide a current density A₂ on the surface of the object;
c. applying a third constant DC current I₃ in the same direction as I₁ to the electrical circuit for a time period t₃ so as to provide a current density A₃ on the surface of the object;
d. repeating steps e. and f., and optionally step d, until the object is plated with the required profile of the metal

The invention is not limited to the description and examples given herein, but may be varied within the scope of the claims.

### Example 1

Figure 3 is a plan view of a base station filter made of aluminium (approximately 1:1 scale). The filter was first plated with a layer of nickel, using an electroless Ni plating bath as commonly used in the art to a thickness of 2.5 µm. The Ni-plated filter was then subjected to Cu plating, first with a DC current, then under alternating reverse and forward pulses and then with a second DC current:

| | |
|---|---|
| *First DC phase* | ca. 0.5 A/dm² for 60 min |
| *Reverse pulse* | ca. 1.7 A/dm² for 2ms |
| *Forward pulse* | ca. 1.0 A/dm² for 1 ms |
| *Total length of time for which the pulse-plating was applied* | 30 min |
| *Second DC phase* | ca. 0.5 A/dm² for 4 min |

The thickness of the copper layer was measured by X-ray. The measurement points were as follows.
1, 2: On the edge of the filter
3: At a depth of 26 mm in a horizontal plane
4,5: On the bottom of the cavity at a depth of ca. 48 mm, (aspect ratio, (depth/diameter) ca. 1.1)
6,7: In the bottom of a cavity in a resonator rod at a depth of ca. 8 mm, (aspect ratio = 1.1)

The following thicknesses were achieved:

| **Point of measurement** | **1** | **2** | **3** | **4** | **5** | **6** | **7** |
|---|---|---|---|---|---|---|---|
| **Cu (µm) after first DC phase** | 30 | 30 | - | 3.7 | 3.7 | 6 | 6 |
| **Cu (µm) after first DC phase + pulse phase** | 0 | 0 | - | - | - | - | - |
| **Cu (µm) after first DC phase + pulse phase + second DC phase** | 5.1 | 6.8 | 5.7 | 3.5 | 3.6 | 5.7 | 5.9 |

| | | | | | | | |
|---|---|---|---|---|---|---|---|
| (-) = not measured | | | | | | | |

As can be seen, the first DC plating step alone gives a coat of Cu which is very unevenly distributed between the edges (1 and 2) and the bottom (4-7) of the base station filter. Pulse-plating can remove Cu which is deposited on the edges 1 and 2. Application of a further DC step creates a Cu coating which is more evenly distributed between the edges (1 and 2) and the bottom (4-7) than previously known methods.

### Example 2

A typical base station with open cavities was pulse-plated with silver. The platable area of the filter was 48 dm², and filters were racked back to back in order to reduce silver outplating on the backside. A minimum 3.0 µm layer of silver in the bottom of the cavity was required. This requirement was achieved by the pulse-plating process according the present invention in less total process time and with a 28 % reduction in silver consumption compared to conventional DC-plating.
The maximum silver thickness, on the edges was 7 µm for pulse-plating and 15 µm for DC-plating. For the pulse-plating process, 16.2 Ah was applied in the forward direction and 10.9 Ah in the backward direction were consumed i. e. the resulting forward consumption is 5.3 Ah.
For DC-plating 7.4 Ah were consumed.

### Example 3

The pulse-plating process according to the invention works also for very narrow dimensions. As a result, the invented pulse-plating process can also be used for applications on Printed Circuit Boards. The technology can be used in the same manner for via holes as for cavities for microwave filters. Using the procedure of sequential DC and pulse reverse plating, it's possible to receive even thicker metal inside the hole, than on the flat board.

## Claims

1. A method for plating an object with a metal coating, **characterized in that** said method comprises the steps of:
a. bringing the object into contact with a solution comprising metal ions;
b. bringing a counter electrode into contact with said solution comprising metal ions;
c. connecting an electrical circuit between the object and the counter electrode;
d. applying a constant DC current I₁ to the electrical circuit for a time period t₁ so as to provide a current density A₁ on the surface of the object so that the object becomes plated with a metal coating;
e. applying a second constant DC current I₂ In the opposite direction as I₁ to the electrical circuit for a time period t₂ so as to provide a current density A₂ on the surface of the object;
f. applying a third constant DC current I₃ in the same direction as I₁ to the electrical circuit for a time period t₃ so as to provide a current density A₃ on the surface of the object; wherein steps e. and f. may take place in either order;
g. repeating steps e. and f., and optionally step d, until the object is plated with the required profile of the metal,
wherein A₂ is greater than A₃.

2. A method according to claim 1, wherein A₂ is at least 1.5 times greater, at least 1.7 times greater, at least 2 times greater or at least 3 times greater than A₃.

3. A method according to claim 1. wherein A₁ is between 0.1 and 5.0 amperes/dm², preferably between 0.2 and 2.0 amperes/dm² and more preferably between 0.25 and 0.75, amperes/dm².

4. A method according to any of the preceding claims, wherein A₂ is between 0.5 and 5.0 amperes/dm², preferably between 0.5 and 2.0 amperes/dm² and more preferably between 0.5 and 1.75 amperes/dm².

5. A method according to any of the preceding claims, wherein A₃ is between 0.5 and 5.0 amperes/dm², preferably between 0.5 and 2.0 amperes/dm² and more preferably between 0.5 and 1.75 amperes/dm².

6. A method according to any of the preceding claims, wherein t₃ is less than t₂.

7. A method according to any of the preceding claims, wherein t₃ is less than 80% of t₂, preferably less than 70% of t₂, most preferably less than 55% of t₂.

8. A method according to any of the preceding claims, wherein t₂ is between 0.2ms and 10ms, preferably between 1 and 5ms and more preferably between 1.5 and 2.5ms.

9. A method according to any of the preceding claims, wherein t₃ is between 0.1ms and 5ms, preferably between 0.5ms and 2.5ms and more preferably between 0.75ms and 1.25ms.

10. A method according to any of the preceding claims, wherein the object contains one or more cavities.

11. A method according to claim 10, wherein the aspect ratio for the cavity, as defined by the ratio between the diameter (D) and the depth (L) of the largest cylinder which fits in the cavity, is between 0.25 and 3 inclusive, preferably between 0.6 and 2.5 inclusive, more preferably 0.75 and 2 inclusive.

12. A method according to any of the preceding claims wherein the cavity is selectively etched a predetermined distance from the plane defining the opening of the cavity, without the use of a mask.

13. A method according to any of the preceding claims wherein the cavity is selectively etched a predetermined distance from the deepest point of the cavity, without the use of a mask.

14. A method according to any of the preceding claims, wherein the metal is selected from the group consisting of Ag, Au, Cu, Ni, Cr and Zn.

15. A method according to any of the preceding claims, wherein the solution comprising metal ions additionally contains one or more surfactants,

16. A method according to claim 16 wherein the surfactant is selected from the group consisting of non-ionic surfactents.

17. A method according to any of claims 15-16 wherein the surfactant is a substituted alkylene oxide compounds.

18. A method according to any of claims 15-17 wherein the surfactant is nonylphenol ethoxylate.

19. A method according to any of claims 15-18 wherein the surfactant is present in a concentration of between 0.01g/l and 10g/l, preferably between 0.1g/l and 1g/l and more preferably between 0.1 g/l and 0.3g/l.

20. A method according to any of the preceding claims, wherein the solution comprising metal ions additionally contains a polymer.

21. A list of computer-readable instructions, said instructions when loaded Into the memory of a processor connected to a DC power supply cause the processor to vary the current of the power supply according to the pulse sequence of steps d., e., f. and g. of claim 1.

## Patentansprüche

1. Verfahren zum Ausbringen eines Metallüberzugs auf einen Gegenstand, **dadurch gekennzeichnet, dass** das Verfahren die folgenden Stufen umfasst :
a. der Gegenstand wird in Kontakt mit einer Metallionen umfassenden Lösung gebracht;
b. eine Gegenelektrode wird in Kontakt mit der Metallionen umfassenden Lösung gebracht;
c. ein elektrischer Stromkreis wird zwischen dem Gegenstand und der Gegenelektrode hergestellt;
d. ein konstanter Gleichstrom I₁ wird an den elektrischen Stromkreis für eine Zeitspanne t₁ angelegt, so dass sich auf der Oberfläche des Gegenstands eine Stromdichte A₁ ergibt, so dass auf den Gegenstand ein Metallüberzug aufgebracht wird;
e. ein zweiter konstanter Gleichstrom I₂ wird in entgegengesetzter Richtung zu I₁ an den elektrischen Stromkreis für eine Zeitspanne t₂ angelegt, so dass sich eine stromdichte A₂ auf der Oberfläche des Gegenstands ergibt;
f. ein dritter konstanter Gleichstrom I₃ wird in gleicher Richtung wie I₁ an den elektrischen Stromkreis für eine Zeitspanne t₃ angelegt, so dass sich eine Stromdichte A₃ auf der Oberfläche des Gegenstands ergibt; wobei die Stufen e. und f. in beliebiger Reihenfolge ablaufen können;
g. die Stufen e. und f. und gegebenenfalls die Stufe d. werden wiederholt, bis auf den Gegenstand das erforderliche Metallprofil aufgebracht worden ist;
wobei A₂ größer als A₃ ist.

2. Verfahren nach Anspruch 1, wobei A₂ mindestens das 1,5-fache, mindestens das 1,7-fache, mindestens das 2-fache oder mindestens das 3-fache von A₃ beträgt.

3. Verfahren nach Anspruch 1, wobei A₁ 0,1 bis 5,0 Ampere/dm², vorzugsweise 0,2 bis 2,0 Ampere/dm² und insbesondere 0,25 bis 0,75 Ampere/dm² beträgt.

4. Verfahren nach einem der vorstehenden Ansprüche, wobei A₂ 0,5 bis 5,0 Ampere/dm², vorzugsweise 0,5 bis 2,0 Ampere/dm² und insbesondere 0,5 bis 1,75 Ampere/dm² beträgt.

5. Verfahren nach einem der vorstehenden Ansprüche, wobei A₃ 0,5 bis 5,0 Ampere/dm², vorzugsweise 0,5 bis 2,0 Ampere/dm² und insbesondere 0,5 bis 1,75 Ampere/dm² beträgt.

6. Verfahren nach einem der vorstehenden Ansprüche, wobei t₃ weniger als t₂ beträgt.

7. Verfahren nach einem der vorstehenden Ansprüche, wobei t₃ weniger als 80 %, vorzugsweise weniger als 70 % und insbesondere weniger als 55 % von t₂ beträgt.

8. Verfahren nach einem der vorstehenden Ansprüche, wobei t₂ 0,2 ms bis 10 ms, vorzugsweise 1 bis 5 ms und insbesondere 1,5 bis 2,5 ms beträgt.

9. Verfahren nach einem der vorstehenden Ansprüche, wobei t₃ 0,1 ms bis 5 ms, vorzugsweise 0,5 bis 2,5 ms und insbesondere 0,75 bis 1,25 ms beträgt.

10. Verfahren einem der vorstehenden Ansprüche, wobei der Gegenstand einen oder mehrere Hohlräume aufweist.

11. Verfahren nach Anspruch 10, wobei das Seitenverhältnis des Hohlraums, das durch das Verhältnis des Durchmessers (D) zur Tiefe (L) des größten, in den Hohlraum passenden Zylinders definiert ist, 0,25 bis einschließlich 3, vorzugsweise 0,5 bis einschließlich 2,5 und insbesondere 0,75 bis einschließlich 2 beträgt.

12. Verfahren nach der vorstehenden Ansprüche, wobei der Holraum selektiv in einem vorbestimmten Abstand von der die Öffnung des Hohlraums definierenden Ebene ohne Verwendung einer Maske geätzt wird.

13. Verfahren nach einem der vorstehenden Ansprüche, wobei der Hohlraum selektiv in einem vorbestimmtem Abstand vom tiefsten Punkt des Hohlraums ohne Verwendung einer Maske geätzt wird.

14. Verfahren nach einem der vorstehenden Ansprüche, wobei das Metall aus der Gruppe, die aus Ag, Au, Cu, Ni, Cr und Zn besteht ausgewählt wird.

15. Verfahren nach einem der vorstehenden Ansprüche, wobei die Metallionen umfassende Lösung zusätzlich ein oder mehr Tenside enthält.

16. Verfahren nach Anspruch 15, wobei das Tensid aus der Gruppe, die aus nicht-ionischen Tensiden besteht, ausgewählt wird.

17. Verfahren nach einem der Ansprüche 15-16, wobei es sich beim Tensid um eine substituierte Alkylenoxid-Verbindung handelt.

18. Verfahren nach einem der Ansprüche 15-17, wobei es sich beim Tensid um Nonylphenolethoxylat handelt.

19. Verfahren nach einem der Ansprüche 15-18, wobei das Tensid in einer Konzentration von 0,01 g/Liter bis 10 g/Liter, vorzugsweise von 0,1 g/Liter bis 1 g/Liter und insbesondere von 0,1 g/Liter bis 0,3 g/Liter vorliegt.

20. Verfahren nach einem der vorstehenden Ansprüche, wobei die Metallionen umfassende Lösung zusätzlich ein Polymeres enthält.

21. Liste von Computer-lesbaren Anweisungen, wobei die Anweisungen nach Laden in den Speicher eines Prozessors, der an eine Gleichstromquelle angeschlossen ist, den Prozessor veranlassen, den Strom I der stromquelle entsprechend der Pulssequenz der stufen d., e., f. und g. von Anspruch 1 zu variieren.

## Revendications

1. Procédé utilisé pour plaquer une couche de métal sur un objet, **caractérisé par le fait que** ledit procédé comprend les étapes suivantes :
a. Mettre l'objet en contact avec une solution contenant des ions métalliques;
b. Mettre une contre-électrode en contact avec ladite solution contenant des ions métalliques ;
c. Connecter un circuit électrique entre l'objet et la contre-électrode ;
d. Appliquer un courant CC constant I₁ sur le circuit électrique pendant une durée t₁ afin de fournir une densité de courant A₁ sur la surface de l'objet pour que l'objet soit plaqué avec une couche de métal ;
e. Appliquer un deuxième courant CC I₂ constant dans le sens opposé à I₁ au circuit électrique pendant une période t₂, pour fournir une densité de courant A₂ sur la surface de l'objet ;
f. Appliquer un troisième courant CC I₃ constant dans le même sens que I₁ au circuit électrique pendant une période t₃, pour fournir une densité de courant A₃ sur la surface de l'objet ; dans lequel les étapes e. et f. peuvent être réalisées dans n'importe quel ordre ;
g. Répéter les étapes e. et f. et éventuellement l'étape d. jusqu'à ce que l'objet soit plaqué avec le profil de métal requis,
dans lequel A₂ est supérieur à A₃.

2. Procédé selon la revendication 1, dans lequel A₂ est au moins 1,5 fois supérieur, au moins 1,7 fois supérieur, au moins 2 fois supérieur ou au moins 3 fois supérieur à A₃.

3. Procédé selon la revendication 1, dans lequel A₁ est entre 0,1 et 5,0 ampères/dm², de préférence entre 0,2 et 2,0 ampères/dm² et encore de préférence entre 0,25 et 0,75 ampères/dm².

4. Procédé selon l'une quelconque des revendications précédentes, dans lequel A₂ se situe entre 0,5 et 5,0 ampères/dm², de préférence entre 0,5 et 2,0 ampères/dm² et encore de préférence entre 0,5 et 1,75 ampères/dm².

5. Procédé selon l'une quelconque des revendications précédentes, dans lequel A₃ se situe entre 0,5 et 5,0 ampères/dm², de préférence entre 0,5 et 2,0 ampères/dm² et encore de préférence entre 0,5 et 1,75 ampère/dm².

6. Procédé selon l'une quelconque des revendications précédentes, dans lequel t₃ est inférieur à t₂.

7. Procédé selon l'une quelconque des revendications précédentes, dans lequel t₃ est inférieur à 80 % de t₂, de préférence, inférieur à 70 % de t₂, et encore de préférence inférieur à 55 % de t₂.

8. Procédé selon l'une quelconque des revendications précédentes, dans lequel t₂ se situe entre 0,2 ms est 10 ms de préférence entre 1 est 5 ms, et encore de préférence entre 1,5 et 2,5 ms.

9. Procédé selon l'une quelconque des revendications précédentes, dans lequel t₃ se situe entre 0,1 ms et 5 ms, de préférence entre 0,5 et 2,5 ms, et encore de préférence entre 0,75 et 1,25 ms.

10. Procédé selon l'une quelconque des revendications précédentes, dans lequel l'objet comporte une ou plusieurs cavités.

11. Procédé selon la revendication 10, dans lequel le rapport d'aspect de la cavité, tel que défini par le rapport entre le diamètre (D) et la profondeur (L) du cylindre le plus large s'insérant dans la cavité, est entre 0,25 et 3 inclus, de préférence entre 0,5 et 2,5 inclus et encore de préférence entre 0,75 et 2 inclus.

12. Procédé selon l'une quelconque des revendications précédentes, dans lequel la cavité est gravée de façon sélective, à une distance prédéterminée du plan définissant l'ouverture de la cavité, sans utiliser de masque.

13. Procédé selon l'une quelconque des revendications précédentes, dans lequel la cavité est gravée de façon sélective, à une distance prédéterminée du point le plus profond de la cavité, sans utiliser de masque.

14. Procédé selon l'une quelconque des revendications précédentes, dans lequel le métal est choisi dans le groupe composé de Ag, Au, Cu, Ni, Cr et Zn.

15. Procédé selon l'une quelconque des revendications précédentes, dans lequel la solution contenant les ions métalliques contient également un ou plusieurs tensioactifs.

16. Procédé selon la revendication 16, dans lequel l'agent de surface est choisi dans le groupe composé de tensioactifs non-ioniques.

17. Procédé selon l'une quelconque des revendications 15 et 16, dans lequel le tensioactif est un composé substitué d'oxyde d'alkylène.

18. Procédé selon l'une quelconque des revendications 15 à 17, dans lequel le tensioactif est du nonylphénol éthoxylate.

19. Procédé selon l'une quelconque des revendications 15 à 18, dans lequel le tensioactif est présent dans des concentrations comprises entre 0,01g/l et 10 g/l, de préférence entre 0,1 g/l et 1g/l et encore de préférence entre 0,1 g/l et 0,3 g/l.

20. Procédé selon l'une quelconque des revendications précédentes, dans lequel la solution comprenant les ions métalliques contient également un polymère.

21. Une liste d'instructions lisibles par ordinateur, lesdites instructions lorsqu'elles sont chargées dans la mémoire d'un processeur connecté à une alimentation électrice CC faisant que le processeur fait varier le courant I de l'alimentation selon la séquence d'impulsion des étapes d., e., f. et g. de la revendication 1.
